

Oct. 13, 1931.

D. MCK. HEPBURN

1,827,522

STONE ASPHALT ROAD AND METHOD OF PREPARING AND LAYING THE SAME

Original Filed Nov. 3, 1925



Inventor.—  
Donald M. K. Hepburn  
by his Attorneys.  
Hourow & Hourow

## UNITED STATES PATENT OFFICE

DONALD MCKNIGHT HEPBURN, OF PHILADELPHIA, PENNSYLVANIA, ASSIGNOR TO  
AMIESITE ASPHALT COMPANY OF AMERICA, OF PHILADELPHIA, PENNSYLVANIA,  
A CORPORATION OF NEW JERSEY

## STONE ASPHALT ROAD AND METHOD OF PREPARING AND LAYING THE SAME

Original application filed November 3, 1925, Serial No. 66,586. Divided and this application filed March 29, 1926. Serial No. 98,383.

My invention relates to bituminous road surfacing materials or compounds and to the manufacture thereof, and to roads formed therefrom, the said materials being of such character that they can be mixed at the quarry where the stone originates or where the aggregate originates, and can be shipped in railroad cars, or trucks over the highways, and can be laid at the temperature of the air 10 without any further preparation, or may be held in storage to be employed at any future time without further preparation. In accordance with the invention the stone or other aggregate is dried and cleaned and prepared 15 for the storing or absorption of a solvent therein before the aggregate comes into contact with the bitumen which is to be used as a binder. This drying and cleaning is done without substantially heating the stone or 20 aggregate and thereafter the solvent is added. After the solvent has been absorbed by the stone, the latter is mixed with the bitumen. The solvent contained in the stone is then 25 slowly absorbed by the cold bitumen which is by this means maintained in a plastic condition. The thorough drying of the stone by my process gives me ample capacity of storing the amount of solvent required to handle the material at the temperature of the air, 30 and the reabsorption of the solvent from the stone into the bitumen extends over a period of many days or even weeks. The material manufactured by this method can thus be shipped long distances and successfully un- 35 loaded and laid in place at the temperature of the air. I have in actual practice shipped the material hundreds of miles, taking ten days or more in transit, and have experienced no trouble in unloading or laying. The ma- 40 terials permit the road surface to be produced with any finish or texture desired for non-skid surfaces.

The principal object of the invention, then, 45 is to provide a slow setting bituminous stock material for road making or surfacing which material is adapted to be transported and laid at atmospheric temperatures and without any preliminary heating.

50 Further objects of my invention will be ap-

parent from the following specification and claims.

The drawing is a diagrammatic view of an apparatus by means of which the manufacture of my improved road composition is 55 facilitated.

Referring to the drawing, 1 represents a revolving drum which is adapted to serve as a cleaner and dryer for the crushed rock or other aggregate which is to be used. As illustrated this drum is inclined to enable the material to progress through it. Suitable means, such as a motor 2, is provided for rotating the drum.

An elevating conveyer 3 is provided for delivering the crushed rock or aggregate to the receiving end of the drum. Before being delivered to the conveyer the rock or other aggregate is suitably graded as to size by screens or other devices which are not shown.

From the drum 1 the aggregate is discharged through a chute 4 into a weighing hopper 5. From the weighing hopper the aggregate is discharged into a suitable mixer 6 which may be provided with a steam-jacket 75 7. From the mixer the material can be discharged into a suitable transporting means, such as a railway car 8.

Air can be supplied to the lower end of the drum 1 by means of a suitable fan 9. 80 For heating the air delivered by the fan, or at least some of the air, I provide a suitable heater which is shown as being an oil burner 10. Preferably I heat only a portion of the air supplied to the fan and I, therefore, provide a funnel 11 through which the heated air is delivered, other air being drawn into the fan around the funnel.

In practicing my improved method, the stone is delivered by the conveyer 3 into the 90 drum 1. By reason of the rotation of the drum, the aggregate is caused to slowly progress downward through the drum, and on doing so it is acted upon by the air delivered by the fan 9. In practice I have found that 95 a large fan is desirable, and for a drum four feet in diameter I prefer a fan having a capacity of approximately 140,000 cubic feet of air per minute. This large volume of air flowing through the drum in opposition to 100

the movement of the aggregate removes all dust and small particles from the aggregate thus thoroughly cleaning it.

The air is used as a drying medium for the aggregate as well as a cleaning medium therefore, and to facilitate the drying action the air is or may be slightly heated. The heating means for the air has already been described, and it will be understood that the fan serves to draw in a large volume of air directly from the atmosphere, and also serves to draw in a smaller volume of highly heated air through the funnel 11. In ordinary practice, I have found that approximately one cubic foot of heated air should be drawn through the funnel for each twenty cubic feet of air drawn directly from the atmosphere. The heated air and the atmospheric air are thoroughly mixed by the fan with the result that the air mixture delivered into the drum is at a temperature only slightly above that of the atmosphere. I prefer to so control the temperature of the air delivered to the drum that the aggregate will not be raised more than six or seven degrees above the atmospheric temperature. I have found that in dry clear summer weather I can eliminate the burner for artificially heating the air, the required drying of the stone being effected by the atmospheric air without heating.

By means of the weighing hopper definite batches of the aggregate of predetermined weight can be delivered to the mixer 6, and from the foregoing description it will be seen that the aggregate thus delivered has been thoroughly cleaned and thoroughly dried without, however, having the temperature thereof raised much above the atmospheric temperature. This avoidance of any substantial increase in the temperature of the aggregate is important for a reason which will presently appear.

As soon as a batch of the aggregate is delivered into the mixer, which is in operation, I add to the aggregate a suitable material which is adapted to serve as a solvent for the asphalt or other bitumen which is to be subsequently added. This solvent should be a slowly volatile one such as kerosene or other oil having a flash test, or evaporating temperature, ranging from 120 degrees F. to 150 degrees F. It will be seen that I select a solvent which will not rapidly evaporate at atmospheric temperature, and which, therefore, will not within a reasonable time be caused to evaporate to any appreciable extent by reason of the contact with the aggregate which, as already stated, is at only a few degrees above the atmospheric temperature. The amount of solvent which is added is carefully predetermined by test so that there will be no excess beyond what can be retained and absorbed by the thoroughly dried and slightly porous surfaces of the stone. I have found that when the stone

is thoroughly dried, as described, a considerable amount of solvent can be absorbed thereby, and the operation of the mixer is continued until all of the surfaces of the aggregate are thoroughly saturated with the solvent and until the solvent is completely absorbed.

After the solvent has been absorbed, I then preferably add a substance which serves to toughen or thicken the bitumen. This substance is preferably hydrated lime and I add from one-half to one percent by actual weight. The mixing is continued until a thoroughly homogeneous mass is produced, with the lime uniformly distributed as a surface coating over the pieces of stone or aggregate. I have found by actual practice that either caustic lime or hydrated lime will produce the same results but, inasmuch as the caustic lime is harder to handle, I prefer to use the hydrated lime.

I then add the required quantity of the bituminous binder which has been previously heated to a temperature of approximately 250 degrees F. or more. Preferably I use from 7½ to 8% by weight of bitumen for the base course material; 9 to 10% for the wearing course material; and 3½ to 4% for the sealing course material. The mixing of the bitumen with the aggregate is continued until all pieces of the aggregate have been thoroughly coated. It will be understood that the heating of the bitumen is primarily for the purpose of more easily securing the required uniformity of mixture and the required uniformity of the distribution of the bitumen over the surfaces of the pieces of stone or aggregate. This heating is not for the purpose of facilitating the subsequent laying of the material, as the material is allowed to become cold before being laid.

The steam-jacket may be used for the purpose of maintaining the heat of the bitumen during the final mixing operation, but is not used during the preliminary mixing operations when the solvent and the lime are added. After the mixing with the bitumen has been completed the mixture is then discharged from the mixer into the railway car or other transporting means.

The hydrated lime which I add to the mixture of my material is used to toughen the binder, particularly at the points of contact with the stone. This also increases the thickness of the bitumen on the individual stones of the aggregate, a result that is very beneficial and desirable. The lime, being added before the bitumen is added to the mix, is very uniformly distributed throughout the entire mass.

According to prior practice, there are three methods of establishing a bond between the aggregate and the bitumen: first, the emulsion method in which the bitumen is emulsified with water; second, the heating of both

the aggregate and the bitumen to about 275 degrees F.; and third, the cold methods of combining the aggregate and bitumen by thinning the latter with a solvent. In the emulsifying method, the aggregate absorbs a large quantity of the water or, in other words, becomes saturated. As the result of this method a comparatively thin coat of bitumen is left on the aggregate, and the mixture has a very temporary life, with a relatively poor bond between the bitumen and the aggregate. By the hot mix method the heat, which is applied to both the aggregate and the bitumen, is used as a distributing agent to keep the material plastic; and the result is that the material must be placed and compacted in the pavement at a high temperature. By the method wherein the solvent is added to the asphalt as a distributing agent, sufficient solvent must be added to handle the asphalt cold. This results in too thin a coat on each individual stone in the aggregate.

From the foregoing it will be apparent that my improved composition differs radically from prior practice in that I neither apply heat to the entire mass to effect distribution nor add a liquefier to effect distribution. I apply heat only to the bitumen, and mix this heated bitumen with cold aggregate in order to obtain a thick coat of bitumen which is chilled in coming into contact with the aggregate. This gives me a thicker coating of asphalt on the individual pieces of aggregate than could be obtained with hot stone. I store the solvent in the stone so that it is not used at all as a fluxing material or liquefier to aid in coating the stone. The solvent having been stored or absorbed in the aggregate before coating and the asphalt having been chilled when coated on the stone, I have a physical condition of the bitumen that holds the heavy coating on the stone. This bitumen, now being cold and far below the melting point thereof, is slowly attacked by the solvent and, due to the fact that the bitumen and stone are cold, the action of the solvent is retarded and this facilitates the unloading and laying of the material days after the material has been mixed. I find in actual practice that the slow absorbing of the solvent by the bitumen tends to draw the bitumen further into the surface of the stone. Any solvent that is absorbed by the bitumen must be replaced by the bitumen penetrating the pores of the stone occupied by the solvent. This not only retards the action of the solvent but also increases the bond between the stone and the bitumen.

In case additional heat is needed in the final mixing to produce a uniform coating of the bitumen on the aggregate, the steam-jacket of the mixer is used. By this method the bitumen absorbs the heat first and the minimum amount required is used, so as not to defeat the advantage gained by using the cold ag-

gregate. In this way I get a thorough coating without the use of a liquefier in the bitumen or heat in the aggregate.

As the material in forming a road is all laid at the temperature of the air, uniform compression is obtained throughout the entire mass. As admitted by experienced pavement engineers, no road rolling in a short space of time by a mechanical roller having a wide contact with the pavement can roll a pavement material to ultimate compression. With my method of manufacture, advantage is taken of the traffic over the road to compact the road and bring it to ultimate compression, as the material is in its original cold and plastic condition so that it can benefit by the compression of traffic.

I claim:

1. The method of mixing a bituminous paving composition, which consists in taking a stone aggregate, subjecting said aggregate to a current of air carefully regulated as to temperature so as to thoroughly dry the aggregate without materially increasing its temperature, thereafter applying to the stone a bitumen solvent, and subsequently adding bitumen to the aggregate.

2. The method of mixing a bituminous paving composition, which consists in taking graded pieces of stone constituting an aggregate, passing thereover a large volume of air to dry them and remove all dust and fines without materially elevating the temperature of the stone, applying to the said pieces of stone a volatile bitumen solvent, and subsequently adding bitumen to the aggregate.

3. The method of mixing a bituminous paving composition, which consists in subjecting graded pieces of stone constituting an aggregate to a current of heated air to dry them and remove all dust and fines, the heat being controlled to avoid heating the stones substantially above atmospheric temperature and the air being in large volume to facilitate the drying operation, applying to the said pieces of stone a bitumen solvent, and immediately adding heated melted bitumen to the aggregate which is maintained at substantially atmospheric temperature until engaged by the bitumen.

DONALD McKNIGHT HEPBURN.

120

125

130